

Aug. 25, 1953

P. F. BRUINS

2,649,624

METHOD OF PRODUCING SISAL FIBER AND WAX

Filed April 5, 1949



FIG. 1



FIG. 2



FIG. 3



FIG. 4

INVENTOR.  
PAUL F. BRUINS  
BY  
Mock & Beum  
ATTORNEYS

## UNITED STATES PATENT OFFICE

2,649,624

METHOD OF PRODUCING SISAL  
FIBER AND WAX

Paul F. Bruins, Douglaston, N. Y., assignor, by  
mesne assignments, to Christian Missions  
Foundation, Inc., New York, N. Y., a corpora-  
tion of New York

Application April 5, 1949, Serial No. 85,494

9 Claims. (Cl. 19—7)

1

My invention relates to a new and improved method of separating sisal wax from sisal leaves, a new and improved method of separating the sisal fiber from the sisal leaves, and a new and improved sisal wax.

The sisal leaf is a spine-shaped leaf whose length is in a range of 0.9 meter to 1.5 meters (3 feet to 5 feet) and whose weight is in a range of 0.545 kilogram to 1.135 kilograms (1 pound to 2.5 pounds). This leaf has an aqueous pulp, and the leaf consists of substantially 80% by weight of water, nearly all of which is in this aqueous pulp.

Heretofore, the sisal leaf has been treated by conveying it to scraping or decorticating drums, as by means of a chain conveyor. These decorticating drums exert pressure and crush the leaves and thus remove the aqueous pulp from the leaves. The machine thus separates the sisal leaves from the aqueous pulp, and also separates the sisal fibres from the leaves. According to this old method, the sisal wax is intermixed with the aqueous separated pulp, which contains nearly all the original water of the leaf. This mixture of pulp and sisal wax is then dried until it is wholly or substantially free from water. The dry mixture of water and pulp residue is then treated with a solvent for the sisal wax, which also dissolves fats, oils, and resins. The solvents which have been used include the chlorinated hydrocarbons, such as trichlorethylene.

When a crude or initial sisal wax is thus extracted from the dry mixture of sisal wax and pulp by the old method, such crude sisal wax has usually at least 50% by weight of resin impurity, and at least 5% by weight of fat and oil impurity. Such extracted crude sisal wax also has black color impurities, which cannot be separated from the crude sisal wax by known, standard decolorizing methods.

These color impurities and other impurities, such as soft and smeary waxes, are originally in the aqueous pulp of the leaf. According to this method, the uncrushed and undecorticated leaf is treated on its surface with a solvent for sisal wax, so that the color bodies and the soft and smeary waxes are substantially not extracted from the aqueous and uncrushed pulp by the solvent.

Such initial or crude sisal wax which is extracted by the old method, and which includes said soft and smeary waxes and said color bodies, is of an amorphous structure.

According to my new and improved method, I treat the sisal leaves, prior to separating the pulp from the leaves, and prior to decorticating the leaves. The leaf thus has its fibre and all or substantially all of its original pulp content when it is treated, and it preferably has all or substantially all of its original water content when

it is treated. The leaf is thus treated while it has its original structure of pulp, cuticle and fibre.

I contact the leaf while it is in said condition and while it has said original structure, having all or substantially all of its pulp and water with a solvent for the sisal wax. This solvent is optionally and preferably anhydrous or substantially anhydrous. This solvent is also optionally and preferably immiscible with water, or substantially immiscible with water. The solvents which I use are exemplified by trichlorethylene, perchlorethylene, carbon tetrachloride and other chlorinated hydrocarbons.

The formula of trichlorethylene is  $C_2HCl_3$  or  $CHClCCl_2$ . It has a boiling point of  $86.7^\circ C$ .

The formula of perchlorethylene, also designated as tetrachlorethylene, is  $CCl_2CCl_2$ . It has a boiling point of  $121^\circ C$ .

The formula of carbon tetrachloride is  $CCl_4$ . It has a boiling point of  $76.74^\circ C$ .

The invention is not limited to the use of chlorinated hydrocarbons, although these are preferred.

The sisal leaf, in said original condition and structure, is preferably contacted with the selected solvent while said solvent is in vapor form, at or a little above the boiling point of the respective solvent. I include the removal of the sisal wax by contact of the sisal leaf with the liquid solvent, which is optionally and preferably heated to a suitable temperature, which may be close to its boiling point, but I prefer to use the solvent in vapor form.

The sisal leaf, while said leaf has its original structure, may be thus contacted with the solvent vapor or liquid in an open tank or vessel, whose pressure is that of the external atmosphere. The sisal leaf, while it has its original structure, may be thus contacted with the vaporized solvent or the liquid solvent in a closed tank or vessel, which may have any desired internal pressure, either above or below standard atmospheric pressure of 760 millimeters of mercury.

I prefer to use an open tank or vessel, such as a tank or vessel open at its top, which contains a pool of the liquid solvent at its bottom, and a heater for heating and vaporizing the solvent, so that its vapor fills the tank or vessel to a selected height, below the top of the tank, above the liquid solvent. This tank or vessel is cooled at its top part, so that the vaporized solvent condenses into liquid at a suitable height, and the liquid solvent drops back into the pool of liquid solvent.

I immerse each leaf in the vaporized solvent during a suitable extraction period. Thus, if I use vaporized trichlorethylene, the extraction period is one to two minutes. During the extraction period, the vapor of the solvent con-

denses on the sisal leaf, due to the high water content of the sisal leaf. I prefer to use a solvent whose boiling point is below 100° C., so that the vaporized solvent produces little or no vaporization of the water of the sisal leaf during the extraction. The solvent vapor thus condenses into liquid solvent on the sisal leaf, and the liquid solvent dissolves the sisal wax. This liquid solution of the sisal wax drops back into the pool of liquid solvent at the bottom of the vessel.

At the end of the extraction period, all or substantially all of the sisal wax is removed from the sisal leaf, and such leaf retains the sisal fibre and all or substantially all of the original pulp, including the water of the pulp. The improved method therefore does not substantially extract the soft and smeary waxes and the color bodies of the aqueous pulp.

Due to the thickness of the sisal leaf, such leaf is not heated through-and-through to the temperature of the vaporized solvent. Thus, if I use vaporized trichlorethylene at or a little above its boiling point of 86.7° C., I estimate that the average through-and-through temperature of the sisal leaf is substantially 49° C. The outer surface of the leaf is heated to a higher temperature than its interior.

While the sisal leaf is thus being dewaxed, it is held vertical or inclined, so that the condensed solvent and its dissolved sisal wax can drip readily off the leaf. There is no loss of solvent in the extraction tank, because its vapor is condensed below the top of the tank.

The leaf becomes limp and softer, due to the treatment thereof. At the end of the dewaxing period, it is free or substantially free from the solvent, because the condensed solvent drops continuously off the leaf.

I then pass the dewaxed and heated and limp sisal leaf immediately to the scraping or decorticating wheels or drums, which remove the sisal fibre in the usual manner while the leaf is hot and limp. Due to the dewaxing and the elevated temperature of the limp sisal leaf, it requires less vigorous mechanical working to remove the sisal fibre. The tensile strength of the sisal fibre is thus improved.

I thus secure an initial or crude sisal wax which has a chocolate-brown color, which is much lighter in color than the crude sisal wax secured according to the old method. This crude sisal wax is substantially free from objectionable impurities which are retained in the aqueous pulp, because I treat the leaf while it has its uncrushed aqueous pulp. As compared with 50% by weight of resin impurity and 5% by weight of fat and oil impurity in a crude sisal wax made according to the old method, the improved crude sisal wax usually has a maximum of 25% by weight of these impurities. By reason of the relatively light color of the improved crude sisal wax, and its relatively high purity, such improved sisal wax can be used for many purposes without any additional treatment, and it can be refined and decolorized if desired, at relatively low cost. For example, this initial or crude sisal wax can be used without additional treatment in shoe polishes, floor polishes, carbon paper, etc., as a substitute for carnauba wax.

As another marked advantage, the initial or crude sisal wax which I produce, is free from certain dark color impurities which are extracted from the dry sisal pulp according to the old method. These objectionable dark impurities

cannot be removed by the known decolorizing methods.

Hence the refined sisal wax which I produce from the initial or crude sisal wax, has a much lighter color than the refined sisal wax made from crude sisal wax which has been extracted according to the old method. The refined sisal wax made from the improved crude sisal wax, can be used as a substitute for the highest grades of carnauba wax and other waxes for many purposes.

It is well-known to degrease metal objects by contacting them with the vapor of trichlorethylene and other fat solvents, and apparatus for this purpose is well-known and hence requires no specific description herein. Such apparatus is disclosed, for example, in Dinley U. S. Patent No. 2,036,261; Dinley U. S. Patent No. 2,028,759; Wolff U. S. Patent No. 1,171,698; Robertson U. S. Patent No. 1,907,875; and Robertson U. S. Patent No. 1,911,928.

Fig. 1 is a microphotograph of the initial or crude sisal wax which is produced according to my method, prior to subsequent refining or decolorizing or bleaching. This microphotograph represents a magnification of 250 diameters and it was taken by transmitted light through a thin layer of said sisal wax, which was deposited on a glass slide from a solution of said sisal wax in carbon tetrachloride. This microphotograph shows a definite crystalline structure of the initial or crude sisal wax which is produced according to my method, prior to any subsequent refining or decolorizing or bleaching;

Fig. 2 is a microphotograph similar to Fig. 1, which illustrates the structure of the initial or crude sisal wax which has been produced according to the old method. Fig. 2 indicates an amorphous structure.

Fig. 3 is a photograph whose left picture shows the color of a film of initial or crude sisal wax made according to the old method, and whose right picture shows the color of a film of initial or crude sisal wax made according to my method, prior to any subsequent refining or decolorizing or bleaching. These photographs were taken of thin layers of the respective sisal waxes, which were deposited on respective glass slides by dipping the respective glass slides into the respective molten waxes. It is clear that the improved crude or initial sisal wax made according to my method, prior to refining or decolorizing or bleaching, has a much lighter color than the corresponding crude or initial sisal wax which has been made according to the old method; and

Fig. 4 corresponds to Fig. 3 save that the layers of the respective sisal waxes were deposited on glass slides from a solution of the respective initial or crude sisal waxes in carbon tetrachloride. As also indicated in Fig. 3, the improved crude or initial sisal wax made according to my method, prior to subsequent refining or decolorizing or bleaching, has a much lighter color than the crude or initial sisal wax made according to the old method.

Specimens of these microphotographs are attached to and made a part of this application.

#### Separation of crude sisal wax from the solvent

The initial or crude sisal wax has a melting point of 85-90° C. As the pool of solvent in the bottom of the extraction tank or vessel takes up the sisal wax, the solution of sisal wax reaches a selected concentration. The solution is removed continuously or in batches from the pool.

said solution is filtered to remove dirt and other suspended solids, and said solution is led through a conventional vaporizing and solvent-recovery mechanism. In this mechanism, the solvent is vaporized and thus separated from the dissolved sisal wax. The separated and pure vaporized solvent is then condensed and led back to said pool of solvent.

The temperature of this mechanism is above the melting point of the initial or crude sisal wax, which is thus recovered in molten form, from which it is allowed to solidify. This solidified crude sisal wax can be subjected, if desired, to one or more additional steps.

#### Decolorizing the crude sisal wax

##### EXAMPLE 1

5 parts by weight of activated decolorizing clay and 1 part by weight of activated decolorizing carbon are added to 100 parts by weight of the initial or crude sisal wax, which is maintained at a temperature of 100° C.-150° C. The mixture is agitated for 30 minutes to one hour, maintaining said temperature.

The decolorized sisal wax is then separated in molten form from the clay and carbon by filtration or other means.

##### EXAMPLE 2

The decolorizing agent is lignin, of the type which is recovered in the kraft paper process. In this kraft paper process, chipped wood is cooked under pressure with a mixture of caustic soda and sodium sulfide. The resultant cook liquor is acidified to recover the lignin. Five parts by weight of such lignin is mixed with 100 parts by weight of the crude molten sisal wax at 130° C.-140° C., and the mixture is agitated at said temperature for one hour.

The resultant mixture is then treated according to Example 1.

These decolorizing methods use decolorizing agents of the adsorbing type.

The above decolorizing steps produce a sisal wax which has a brown to tan color which is much less dark than in the initial crude wax. Since I do not extract objectionable dark coloring matter from the dry pulp of the sisal leaf according to my method, this decolorizing produces a wax of much lighter color than when the initial crude sisal wax is made according to the old method.

#### Bleaching or chemical decolorizing

For this purpose, I can use sodium hypochlorite, bleaching powder, organic peroxides such as benzoyl peroxide, inorganic peroxides, sulfuric acid, other acids, and other chemical bleaching or decolorizing agents.

I can use these chemical agents before or after treatment with the activated clay, activating carbon, and other adsorbing decolorizing agents.

#### Removal of fats and oils from the crude sisal wax

After the crude sisal wax has been separated from the solvent, such wax is passed in finely divided form into a pool of anhydrous acetone which is kept at a temperature of 25° C., with constant stirring. The crude sisal wax may be in finely divided solid form when it is added to the acetone. The crude sisal wax may be in molten form, and it is added slowly to the pool of acetone to be solidified in fine particles in said pool. The acetone dissolves the fats and oils of the crude sisal wax, without dissolving the

sisal wax or its resin impurity. For this purpose I can use other selective solvents at ordinary room temperature of 20° C.-25° C. such as higher-boiling ketones, diethyl ether, and other higher-boiling point ethers.

I optionally prefer to remove the fat and oil impurities from the crude sisal wax, before removing the resin impurities.

The partially purified sisal wax is separated 10 from the selective solvent by filtration, centrifuging, settling, or any other suitable method.

#### Removing resin impurities from the crude sisal wax, after removing the fat and oil impurities

15 The sisal wax is soluble in hot alcohols, such as methanol, ethanol, isopropanol, other suitable monohydric alcohols and other solvents, in which the resin impurity is insoluble.

The partially purified sisal wax is mixed with 20 the selective solvent at suitable temperature, such as 50° C., if methanol is used in order to dissolve the sisal wax, without dissolving the resin. The solution of the sisal wax in the solvent is separated from the undissolved resin, and the solution of the sisal wax is cooled to 20° C.-25° C. or below, to separate the sisal wax from the solvent.

The residual solvent in the purified sisal wax is driven off.

I can treat this purified sisal wax with the adsorbing and chemical decolorizing agents, and this is preferred.

Microscopic observation fails to show any difference in structure between sisal fibre separated from the sisal leaf according to my method, as compared with the old method.

Tensile tests have shown that an improved sisal fibre is produced by decorticating the de-waxed sisal leaf.

|                                                 | Old Method<br>Fibre from<br>Untreated<br>Sisal Leaves,<br>Grams | New Method<br>Fibre from<br>Dewaxed<br>Sisal Leaves,<br>Grams |
|-------------------------------------------------|-----------------------------------------------------------------|---------------------------------------------------------------|
| 45 Tensile Strength of the Full Length<br>Fibre | 886                                                             | 931                                                           |
| Tensile Strength of the Lower Third             | 1,122                                                           | 1,182                                                         |
| Tensile Strength of the Middle Third            | 1,133                                                           | 1,242                                                         |
| Tensile Strength of the Upper Third             | 770                                                             | 736                                                           |

55 If a crude sisal wax which has been produced according to the old method, is subjected to the above-mentioned decolorizing agents as above stated, the resultant sisal wax is much darker in color than when the starting material is a crude sisal wax produced according to my method. This is because the solvent extracts certain black impurities from the dry pulp, which the solvent does not extract from the aqueous pulp. The improved decolorized sisal wax is therefore substantially free from the dark impurities of dry sisal pulp.

60 The improved sisal wax retains its crystalline structure, when the improved sisal wax is treated as above described.

65 I have described a preferred embodiment of my invention, but numerous changes and omissions and additions and substitutions can be made without departing from its scope.

I claim:

70 1. A method of separating sisal wax from a sisal leaf, which consists in contacting the surface of said leaf with a solvent of sisal wax and extracting and dissolving the sisal wax of said leaf in said solvent and removing said solution from said leaf, said leaf being thus contacted

with said solvent and said solution being removed from said leaf while said leaf has its fibre and also has its aqueous pulp in uncrushed form, said solvent extraction being substantially confined to said surface to retain in said uncrushed aqueous pulp substantially all of its wax and color bodies which are soluble in said solvent.

2. A method of separating sisal wax from a sisal leaf, which consists in contacting the surface of said leaf with the vapor of a solvent of sisal wax, condensing said vapor in liquid form on said surface and extracting and dissolving the sisal wax of said leaf in said condensed liquid solvent and removing said solution from said leaf, said leaf being thus contacted with said vapor and said condensed liquid solvent and said solution being removed from said leaf while said leaf has its fibre and also has its aqueous pulp in uncrushed form, said solvent extraction being substantially confined to said surface to retain in said uncrushed aqueous pulp substantially all of its wax and color bodies which are soluble in said solvent.

3. A method of separating sisal wax from a sisal leaf, which consists in contacting the surface of said leaf with a solvent of sisal wax and extracting and dissolving the sisal wax of said leaf in said solvent and removing said solution from said leaf, said leaf being thus contacted with said solvent and said solution being removed from said leaf while said leaf has its fibre and also has its aqueous pulp in uncrushed form, said solvent extraction being substantially confined to said surface to retain in said uncrushed aqueous pulp substantially all of its wax and color bodies which are soluble in said solvent, said solvent being substantially immiscible with water.

4. A method of separating sisal wax from a sisal leaf, which consists in contacting the surface of said leaf with the vapor of a solvent of sisal wax, condensing said vapor in liquid form on said surface and extracting and dissolving the sisal wax of said leaf in said condensed liquid solvent and removing said solution from said leaf, said leaf being thus contacted with said vapor and said condensed liquid solvent and said solution being removed from said leaf while said leaf has its fibre and also has its aqueous pulp in uncrushed form, said solvent extraction being substantially confined to said surface to retain in said uncrushed aqueous pulp substantially all of its wax and color bodies which are soluble in said solvent, said solvent being substantially immiscible with water.

5. A method of treating a sisal leaf, which consists in contacting the surface of said leaf with a solvent of sisal wax and extracting and dissolving the sisal wax of said leaf in said solvent, said leaf being thus contacted with said solvent while said leaf has its fibre and also has its aqueous pulp in uncrushed form, said solvent extraction being substantially confined to said surface to retain in said uncrushed aqueous pulp substantially all of its wax and color bodies which are soluble in said solvent, and then decorticating said leaf while crushing its aqueous pulp.

6. A method of treating a sisal leaf which consists in contacting the surface of said leaf with the vapor of a solvent of sisal wax, condensing said solvent in liquid form on said surface and extracting and dissolving the sisal wax of said leaf in said condensed solvent and removing said solution from said leaf, said leaf being thus contacted with said vapor and said condensed

solvent and said solution being removed from said leaf while said leaf has its fibre and also has its aqueous pulp in uncrushed form, said solvent extraction being substantially confined to said

5 surface to retain in said uncrushed aqueous pulp substantially all of its wax and color bodies which are soluble in said solvent, and then decorticating said leaf while crushing its aqueous pulp.

10 7. A method of treating a sisal leaf, which consists in contacting the surface of said leaf with a solvent of sisal wax and extracting and dissolving the sisal wax of said leaf in said solvent, said leaf being thus contacted with said

15 solvent while said leaf has its fibre and also has its aqueous pulp in uncrushed form, said solvent extraction being substantially confined to said surface to retain in said uncrushed aqueous pulp substantially all of its wax and color bodies

20 which are soluble in said solvent, and then decorticating said leaf while crushing its aqueous pulp, said solvent being heated to a sufficiently high temperature to make said leaf hot and limp at the end of said extraction, said leaf being hot

25 and limp when the decortication of the leaf is begun.

8. A method of treating a sisal leaf which consists in contacting the surface of said leaf with the vapor of a solvent of sisal wax, condensing

30 said solvent in liquid form on said surface and extracting and dissolving the sisal wax of said leaf in said condensed solvent and removing said solution from said leaf, said leaf being thus contacted with said vapor and said condensed solvent

35 and said solution being removed from said leaf while said leaf has its fibre and also has its aqueous pulp in uncrushed form, said solvent extraction being substantially confined to said surface to retain in said uncrushed aqueous pulp

40 substantially all of its wax and color bodies which are soluble in said solvent, and then decorticating said leaf while crushing its aqueous pulp, said vapor being at a sufficiently high temperature to make said leaf hot and limp at the end of said extraction, said leaf being hot and limp when the decortication of the leaf is begun.

9. A method of decorticating a sisal leaf which has its aqueous pulp in uncrushed form, which consists in heating said leaf to at least substantially 50° while removing the sisal wax from said leaf by surface solvent extraction to produce a hot and limp sisal leaf which has substantially all of said aqueous pulp in uncrushed form, and then decorticating said leaf while it is hot and limp by scraping said leaf under pressure while crushing said aqueous pulp.

PAUL F. BRUINS.

60 References Cited in the file of this patent

UNITED STATES PATENTS

| Number    | Name          | Date           |
|-----------|---------------|----------------|
| 2,048,719 | Whitford      | July 28, 1936  |
| 2,372,561 | Elgin         | Mar. 27, 1945  |
| 2,428,813 | Rhodes et al. | Oct. 14, 1947  |
| 2,449,107 | Broeg et al.  | Sept. 14, 1948 |

70 FOREIGN PATENTS

| Number  | Country       | Date          |
|---------|---------------|---------------|
| 575,642 | Great Britain | Feb. 27, 1946 |

OTHER REFERENCES

75 Politzer "Waxes From Sisal Waste," Chemistry and Industry, June 26, 1948, pages 408-409.